

# UNITED STATES PATENT OFFICE.

ROBERT JOYNES BAGGALY, OF NOTTINGHAM, ENGLAND.

## COMPOSITION OF MATERIAL FOR DAMP-PROOF SOCKS OR SOLES FOR BOOTS, &c.

SPECIFICATION forming part of Letters Patent No. 315,885, dated April 14, 1885.

Application filed January 31, 1885. (No specimens.) Patented in England January 15, 1883, No. 230.

*To all whom it may concern:*

Be it known that I, ROBERT JOYNES BAGGALY, manufacturer, a subject of the Queen of England, residing at Nottingham, England, 5 have invented a new and useful Improved Composition of Materials for Damp-Proof Socks or Soles for Boots and Shoes, and method of preparing or manufacturing the same, (for which I have obtained a British patent, No. 10 230, dated January 15, 1883,) of which the following is a specification.

The said invention relates to the manufacture of an improved composition of materials for making damp-proof socks or soles for boots 15 and shoes in an improved, economical, more satisfactory, and convenient manner than heretofore.

Hitherto socks or soles for boots and shoes have been principally manufactured from the 20 bark of the cork-tree, commonly known as "cork," which must necessarily be cut the way of the grain of the wood, so as to obtain the requisite size. Such socks or soles are generally defective by reason of the numerous 25 pores or minute holes or flaws in the wood or material, which eventually allow the wet or damp to reach the feet of the wearer.

The object of my present invention is therefore to produce socks or soles manufactured 30 from a material or composition of materials devoid (or nearly so) of the porosity of sheets of cork, and consequently better adapted to protect the feet against the evil effects of damp or wet. The said improved composition of 35 materials for damp-proof socks or soles for boots and shoes is prepared by reboiling boiled linseed-oil, (or other suitable drying-oil,) with the addition of caustic lime and borax, in the proportion of one pound weight of each 40 of them to one hundred-weight of oil. The reboiling is continued until the compound, when cold, is about of the consistency of putty, and when the compound is cold there is kneaded into it half a pound more caustic lime, one 45 ounce of essential oil of almonds, and two

pounds of flowers of sulphur, with finely pulverized or ground cork, in the proportion of one and one-quarter hundred-weight of cork to one hundred-weight of the compound. The compound is next passed between rollers, and 5 by suitable pressure spread upon fleece, felt, animals' skins, or other suitable non-conductor of heat, which is fed to the rollers in the required proportion. The improved compound is thus formed into sheets or lengths of compact material having on one side of the material a warm covering of some suitable non-conductor of heat, and when these sheets or lengths of material are dry they may be cut or stamped out, either by hand or machinery, 6 into shapes suitable for socks and soles of boots and shoes, and any subsequent stitching or binding operations are rendered unnecessary.

The improved material may also with great 6 advantage be used in the manufacture of boots and shoes, a layer of the material being placed between the outer and inner soles of the boots and shoes. The material is also applicable for making the bodies of hats when covered 7 with suitable material.

It is obvious that by varying the ingredients or substituting or adding others various compounds of cork and oil may be formed which may be employed for forming sheets or lengths 7 of materials from which damp-proof socks or soles for boots and shoes may be manufactured; but I preferably employ the compound hereinbefore described, as being better adapted for the purpose than any other composition. 8

I claim—

The herein-described composition of matter, consisting of oxidized linseed-oil, caustic lime, borax, essential oil of almonds, flowers of sulphur, and pulverized or ground cork, in the 8 proportions substantially as specified.

ROBERT JOYNES BAGGALY.

Witnesses:

WALTER HICKLING PERRY,  
LOCK MOORE.